

## UNITED STATES PATENT OFFICE

LEO WALLERSTEIN, OF NEW YORK, N. Y., ASSIGNOR TO WALLERSTEIN COMPANY, INC.,  
OF NEW YORK, N. Y., A CORPORATION OF NEW YORK

## PROCESS OF DEGUMMING SILK

No Drawing.

Application filed January 7, 1928. Serial No. 245,263.

This invention relates to certain improvements in a process for degumming silk.

In a prior patent issued to me No. 1,644,764, dated October 11, 1927, I have disclosed a process for degumming silk which consists in a treatment of the silk, under suitable conditions as to temperature, etc., with a solution of a proteolytic enzyme, such as papain, which is active in an acid, in a 10 slightly alkaline, and in a neutral medium, and in a co-pending application Serial No. 165,491 I have disclosed the treatment of such enzyme solution with an activator, such as potassium cyanide, which reduces the 15 amount of the enzyme necessary to effect the desired degumming of the silk, and also effects a more complete and quicker action of the enzyme.

It is the especial object of the present invention to provide a process which will have the desired degumming effect on the silk, but in which an activator is employed with the enzyme solution which is substantially non-poisonous and, therefore, safe and easy 25 to handle, and which at the same time will have the desired activating effect on the enzyme.

I have discovered that the salts of hydro-sulfurous acid, such for instance as sodium 30 hydro-sulfite or its formaldehyde compound, sodium sulfoxylate, are activators which when used under suitable conditions as to temperature, etc., in the enzyme solution have the desired activating effect on the 35 enzyme, but at the same time are substantially non-poisonous, so that they may be used with safety and with the desired effects.

In carrying out my process, the silk, in skeins or other desired or convenient form, 40 is subjected to a preliminary washing in a weak soap solution or weak alkaline solution. The washed silk is then immersed in a solution or bath of the selected proteolytic enzyme, as for instance papain, at a temperature of 50° C. or above, the silk, after it has been sufficiently degummed, being rinsed and dried.

In carrying out the process of the present invention, I add to the enzyme bath an activator in the form of a salt of hydro-sulfurous 50

acid, which is substantially non-poisonous, the employment of such salt rendering the bath safe to handle and effecting a decrease in the amount of the enzyme used and the desired acceleration of its action.

While various salts of hydro-sulfurous acid may be used and the conditions of use may be somewhat varied, as a specific example I may proceed as follows, using a papain solution as illustrative. The papain 55 bath or solution is prepared in the proportion of one gram of papain of commercial strength to 5 liters of water. To this bath is added a salt of hydro-sulfurous acid, such as sodium hydro-sulfite or its formaldehyde 60 compound, such as sodium sulfoxylate, or both if desired. This activator is added to the bath in amounts which may vary. In actual practice, from 1 to 4 parts of the activator may be used for each part of papain, 65 as for instance for the papain bath specified from 1 to 4 grams of the activator may be added. The whole amount of the activator may be added to the bath at once, or it may be added at different times while the degumming action of the enzyme is taking 70 place, such procedure having been found to be of advantage under certain conditions of use.

By the use of such activator, the time of 75 the desired degumming action of the enzyme is reduced, thus permitting faster working, and the amount of the enzyme proportionately to the amount of the silk treated may be lessened, and at the same time the activator 80 may be safely used and without any deleterious action on the fiber of the silk.

What I claim is:

1. The process of degumming silk which 85 consists in subjecting the silk to the action of a proteolytic enzyme of that type which is active in a neutral, weak alkaline, and a slightly acid medium and which is activated by the presence of a salt of hydro-sulfurous acid until the desired amount of degumming 90 has occurred.

2. The process of degumming silk which 95 consists in subjecting the silk to the action of a proteolytic enzyme of that type which is active in a neutral, weak alkaline, and a 100

slightly acid medium and which is activated by the presence of a sodium salt of hydro-sulfurous acid.

3. The process of degumming silk which consists in subjecting the silk to the action of a proteolytic enzyme of that type which is active in a neutral, weak alkaline, and a slightly acid medium and which is activated by the presence of sodium hydro-sulfite.
- 10 4. The process of degumming silk which consists in subjecting the silk to the action of a solution of papain in the presence of a salt of hydro-sulfurous acid.
- 15 5. The process of degumming silk which consists in subjecting the silk to the action of a solution of papain in the presence of a sodium salt of hydro-sulfurous acid.
- 20 6. The process of degumming silk which consists in subjecting the silk to the action of a solution of papain in the presence of sodium hydro-sulfite.
- 25 7. The process of degumming silk which consists in subjecting the silk to the action of a solution of papain in the presence of sodium hydro-sulfite and sodium sulfoxylate.
- 30 8. The process of degumming silk which consists in subjecting the silk in a bath or solution of papain to which has been added sodium hydro-sulfite in quantities from 1 to 4 parts by weight of the enzyme at a temperature sufficient to maintain the activity of the enzyme.

In testimony whereof, I have hereunto set  
35 my hand.

LEO WALLERSTEIN.

40

45

50

55

60

65